

Dec. 29, 1925.

1,567,143

J. T. HAY

## ANNEALING STEEL SHEETS

Filed Jan. 19, 1925

2 Sheets-Sheet 1



Fig. 1



FIG. 2

*John T. Hay*

By *Grease and Bond*

Attorneys

Dec. 29, 1925.

1,567,143

J. T. HAY

ANNEALING STEEL SHEETS

Filed Jan. 19, 1925

2 Sheets-Sheet 2

Fig. 3



Fig. 4



Inventor

*John T. Hay*

By *Grease and Bond*

Attorneys

## UNITED STATES PATENT OFFICE.

JOHN THOMAS HAY, OF CANTON, OHIO, ASSIGNOR TO UNITED ALLOY STEEL CORPORATION, OF NEW YORK, N. Y., A CORPORATION OF NEW YORK.

## ANNEALING STEEL SHEETS.

Application filed January 19, 1925. Serial No. 3,309.

To all whom it may concern:

Be it known that I, JOHN THOMAS HAY, a citizen of the United States, residing at Canton, in the county of Stark and State of Ohio, have invented certain new and useful Improvements in Annealing Steel Sheets, of which the following is a specification.

The invention relates to the annealing of chrome steel or iron sheets, comprising a chrome alloy of steel or iron which may contain silicon or other alloy elements.

When such sheets are annealed by ordinary methods, there is formed an insoluble scale in the sheet surfaces, which cannot be removed by any known pickling process. Moreover, such sheets are not easily adapted to deep drawing processes.

The objects of the present invention are to provide a method of annealing chrome steel sheets, wherein the scale formed on the sheet surfaces may be removed by pickling; and to produce by the above method a sheet which when finished has a fine grained structure adapted to deep drawing.

These objects may be attained by separately placing the sheets on edge in a heating furnace, after they have been first heated and reduced by rolling, and admitting a quantity of oxygen into the furnace for rendering soluble in a pickling solution the scale formed upon the sheets by the prior rolling and annealing processes or by the instant annealing process, and rapidly and uniformly heating the sheets in the furnace to produce a fine granular structure adapted for deep drawing.

One form of apparatus for carrying out the invention is illustrated in the accompanying drawing, forming part hereof, in which—

Figure 1 is a plan cross section of a heating furnace for carrying out the invention, as on line 1—1, Fig. 2;

Fig. 2, a longitudinal cross-section of the same, as on line 2—2, Fig. 1;

Fig. 3, a transverse cross-section of the same, as on line 3—3, Fig. 2, showing a pile of sheets partially arranged on edge in the furnace; and

Fig. 4, a transverse cross-section of the same as on line 4—4, Fig. 2, showing the sheets arranged on edge in the furnace, as during the annealing process.

Similar numerals refer to similar parts

throughout the several figures of the drawing.

The furnace may be an ordinary sheet heating furnace, including side walls 1 and 2, end walls 3 and 4, and arched top 5, built in any well known manner upon a foundation indicated at 6, and providing an interior which is divided by baffle wall 7 to form a firing chamber indicated by 8 and a sheet chamber indicated by 9; such a furnace being sometimes known as a semi-muffle furnace.

Within the firing chamber 8, a grate 10 is secured, and the end wall 3 is provided with a fire door 11 above the grate, and a draft door 12 below the grate for firing the grate with a fuel indicated at 13, and controlling the combustion of the same. It is to be understood that any other desired form of heating means may be employed in place of the means illustrated.

End wall 4 is provided with a sheet door 14, having an opening and closing mechanism indicated at 15, permitting access to the sheet chamber 9.

A floor 16 preferably having a series of longitudinal notches 16<sup>a</sup> is provided in the sheet chamber and supported by a series of spaced longitudinal flue walls 17 to provide a plurality of flues 18 beneath the floor 16, and in communication with the sheet chamber 9, through apertures 18<sup>a</sup> in the floor.

Flues 18 are directed into a transverse tunnel 19 situated between the end wall 4 and the baffle wall 7, and tunnel 19 communicates by way of side stacks 20 and 21 with the centrally located main stack 22, as shown. A check damper indicated at 23 is provided in the main stack 22 for controlling the gas flow through the stack.

The same furnace may be used to heat the chrome steel sheets 24 before rolling, but as here shown in Fig. 3, a pile of sheets 25 has been first heated, then rolled, and then inserted, preferably singly, through the door 14 into the sheet chamber, and a number of the separate sheets have been placed on edge preparatory to annealing.

In Fig. 4, all the sheets have been placed on edge and are now ready for annealing.

Chrome steel sheets as they come from the rolls have a tightly adhering scale after ordinary annealing in a reducing atmosphere, which scale is insoluble in ordinary pickling

baths. This scale is increased and rendered more insoluble by the annealing process.

By the present method the sheets are preferably heated in the furnace for a period of about twenty minutes, depending upon their thickness, and then the check draft 23 is adjusted to permit a predetermined flow of air through the furnace and around the separated sheets as indicated by the arrows. 10 This flow of air, for a period of about ten minutes, and the constituent oxygen causes the formation upon the sheet surfaces of a scale which is readily soluble in a pickling bath containing sulphuric acid and hydrochloric acid, which acids may be in proportions of 5% of sulphuric and 2% of hydrochloric, as set forth in my Letters Patent No. 1,542,541.

The sheets are thus subject to a hot annealing atmosphere which is first reducing and then oxidizing for a total period of about thirty minutes, at the end of which the sheets have a fine granular structure adapting them to deep drawing.

25 During the heating the sheets are preferably intermittently turned over from one edge to the other to secure a uniform annealing of all parts of the sheet.

I claim:

30 1. The method of annealing chrome steel sheets which includes heating the sheets for annealing in an oxidizing atmosphere to form a soluble scale thereon.

2. The method of annealing chrome steel sheets which includes heating separated sheets for annealing in an oxidizing atmosphere to form a soluble scale thereon.

35 3. The method of annealing chrome steel sheets which includes heating the sheets for annealing in an oxidizing atmosphere, and intermittently agitating the sheets during

the heating period, to form a soluble scale thereon.

4. The method of annealing chrome steel sheets which includes heating the sheets for 45 annealing in a reducing atmosphere and then heating them in an oxidizing atmosphere to form a soluble scale thereon.

5. The method of annealing chrome steel sheets which includes heating the sheets for 50 about ten minutes in an oxidizing atmosphere.

6. The method of annealing chrome steel sheets which includes heating the sheets in a reducing atmosphere and then heating the 55 sheets for about ten minutes in an oxidizing atmosphere.

7. The method of annealing chrome steel sheets which includes heating the sheets in a reducing atmosphere for about twenty minutes and then heating the sheets in an oxidizing atmosphere.

8. The method of annealing chrome steel sheets which includes heating the sheets in a reducing atmosphere for about twenty minutes and then heating the sheets in an oxidizing atmosphere for about ten minutes.

9. The method of treating chrome steel sheets which includes annealing the sheets by heating them in an oxidizing atmosphere 70 to form a soluble scale thereon, and then pickling the sheets in sulphuric and hydrochloric acids.

10. The method of treating chrome steel sheets which includes annealing the sheets by 75 heating them in an atmosphere which is first reducing and then oxidizing to form a soluble solution thereon, and then pickling the sheets.

In testimony that I claim the above, I 80 have hereunto subscribed my name.

JOHN THOMAS HAY.